

# UNITED STATES PATENT OFFICE.

ARTHUR HOWARD HIGGINS, OF LONDON, ENGLAND, ASSIGNOR, BY MESNE ASSIGNMENTS, TO MINERALS SEPARATION NORTH AMERICAN CORPORATION.

## CONCENTRATION OF ORES.

1,236,934.

Specification of Letters Patent. Patented Aug. 14, 1917.

No Drawing.

Application filed September 23, 1914. Serial No. 863,098.

To all whom it may concern:

Be it known that I, ARTHUR HOWARD HIGGINS, a subject of the King of England, residing at 62 London Wall, London, England, have invented certain new and useful

5 Improvements in the Concentration of Ores.

This invention is for improvements in or relating to the concentration of ores and especially to preferential or selective flotation, that is to say, to the separation of different metallic sulfids from one another as well as from gangue when flotation processes are used, and the present invention is in some respects a development from that 10 described in the prior United States Patent to Nutter *et al.*, No. 1067485, issued July 15, 1913.

For the purpose of defining the nature 20 of this invention it is desirable first to discuss the factors which obtain in froth flotation processes and for this purpose attention will be particularly directed to the apparatus of the sub-aerator type defined in the specification of my United States Patent 25 No. 1,155,816, issued October 5, 1915, that is to say, to a flotation apparatus in which the particles in the pulp in a comparatively quiet zone in the upper portion of the flotation vessel are subjected to the 30 action of a continuous stream of innumerable minute gaseous bubbles rising to a froth outlet at the top.

An important factor in froth flotation processes is the tendency of a particle to be 35 wetted by water, and conversely the tendency of a particle to become dry or to become attached to a gaseous bubble. The gangue particles have the greatest tendency to be wetted by water and have the least 40 tendency to be attached to gaseous bubbles. Further, comparing galena and blonde, for example, the particles of galena appear to have the least tendency to be wetted by water or the greatest tendency to become attached to gaseous bubbles, while blonde particles appear to have a somewhat smaller 45 tendency to be attached to gaseous bubbles. Pyrites appear to have a still greater tendency than galena to be attached to gaseous 50 bubbles.

In a flotation process (particularly if carried out in an apparatus of the type above referred to) it is found that another im-

portant factor is the rate at which the different particles fall in water or the weight 55 of the particles in water in relation to their size.

If a pulp contains very fine particles of blonde and galena of the same size, the galena particles will be heavier than the blonde 60 particles in the relation of about 7 to 4 or their weight in water will be in the relation of about 6 to 3. The galena particles will therefore have a much greater rate of fall 65 in water than the blonde particles.

If such a sized product is subjected to a flotation process under conditions suitable for preferential flotation, it is found that the gravity factor predominates and the zinc is floated more readily than the lead. 70

This invention, therefore, lies in a process for the selective separation of the different constituents of an ore by flotation in which the finely crushed ore is sized so as to yield products containing particles of substantially uniform size, whereupon these products are separately treated by a preferential flotation process so as to obtain flotation products relatively high in a certain sulfid 75 on the one hand and residues relatively high 80 in another sulfid on the other hand.

In the original agitation froth apparatus as illustrated in the prior United States Patent to Sulman *et al.*, No. 835120, issued November 6, 1906, for example, the actual 85 formation of the froth took place on the surface of a spitzkasten in which the liquid was comparatively at rest, and the gravity factor played little or no part. In the sub-aerator type of apparatus where the separation 90 does not take place in a spitzkasten, but where the separation of the froth takes place at the top of the agitation and aeration vessel itself, the phenomenon of gaseous flotation is a dynamic one and the gravity 95 factor may be caused to play a considerable part.

Briefly it may be stated that this invention consists in the simultaneous use of the factors of differential gaseous attachment 100 and differential falling power in liquid to secure selective flotation.

In carrying this invention into effect it is found that the conditions most suitable for preferential or selective flotation are as 105 follows:

The frothing agent employed should be partly soluble in water, such as eucalyptus amygdalina, and the proportion employed should be very small (about one or two 5 ounces per ton of ore treated, *i. e.* for four tons of water). Additions of frothing agent may be made during the treatment if it is desired to increase the rate at which the froth is produced, care being taken to avoid 10 excess. In a number of previous patents relating to this subject reference has been made to the use of solutes such as acids, alkalies, and soluble salts to assist the selection of the air bubbles. A process embodying this invention may involve the use of 15 these agents and a simple preliminary test of any particular ore would determine the chemical constitution of the solution to be employed. In most of the experiments 20 which led to the present invention the pulp was alkaline containing about 0.1 to 0.3% of sodium carbonate in solution. Successful results have also been obtained with other salts such as sodium bicarbonate and sodium 25 sulfate.

With regard to sized material, this invention is particularly applicable to finely crushed mixed sulfid ores of the following sizes:  $(-80 + 100)$ ,  $(-100 + 120)$ , or  $(-120 + 150)$ , these sizes being given in meshes to the linear inch according to the standard of the Institute of Mining and Metallurgy. The more closely sized the product is, the more exact is the selective flotation.

35 The following examples illustrate the application of this invention. In each case the test was made in a small laboratory apparatus of the general type described in my United States Patent No. 1,155,816, issued 40 October 5, 1915.

#### Example 1.

The crude ore was crushed and sized and the particular size in this test was  $-120 + 150$  I. M. M. The original assay showed 45 Zn 11.31%, Pb 11.76%. This material was treated in a circuit containing 0.11% of dry sodium carbonate ( $\text{Na}_2\text{CO}_3$ ). There was first added 2.7 ozs. eucalyptus oil per ton 50 of ore and the mixture was agitated 4 minutes and one part of the first concentrates was removed. There was then added 2.7 ozs. eucalyptus per ton of ore and the mixture was agitated for 4 minutes more and 55 the second part of the first concentrates removed. There was then added 5.4 ozs. eucalyptus per ton of ore and the mixture was agitated for 8 minutes and the third part 60 of the first concentrates removed. It was observed that practically all the zinc had been removed. There was then added 3 ozs. per ton of ore of a mixture of Texas oil and wood tar oil, and the mixture agitated for 8½ minutes and the lead concentrate was removed.

The result of these four parts was as follows:

| Proportion of original in concentrate. | Assay of concentrate.                | Recovery.               |
|----------------------------------------|--------------------------------------|-------------------------|
| 4.5%                                   | { 42.3% Zn.<br>6.4% Pb.<br>1.8% Ins. | { 17.0% Zn.<br>2.4% Pb. |
| 9.5%                                   | { 44.8% Zn.<br>2.6% Pb.<br>0.5% Ins. | { 37.8% Zn.<br>2.1% Pb. |
| 6.7%                                   | { 42.9% Zn.<br>9.4% Pb.<br>1.6% Ins. | { 25.5% Zn.<br>5.4% Pb. |
| 15.2%                                  | { 6.2% Zn.<br>67.4% Pb.<br>2.2% Ins. | { 8.3% Zn.<br>86.8% Pb. |

70

75

80

The proportion of tailings was 58.4, assaying 2.0% Zn, 0.6% Pb.

The first three parts form the zinc concentrate of average assay of 43.5% zinc with a recovery of 80.3% of the zinc.

#### Example 2.

Here again the ore was crushed and sized and it was the size  $-120 + 150$  I. M. M. that was treated in this example, and the original assay was 18.89% Zn 14.18% Pb.

The conditions were similar to those in Example 1, except that the proportion of dry sodium carbonate was 0.176% on the water and the additions of eucalyptus were 1.7 ozs. per ton of ore for the zinc concentrates of which there were 2; and 3 ozs. of the mixture of Texas oil and wood tar oil for lead concentrate.

The results were as follows:

| Proportion of original in concentrate. | Assay of concentrate.                 | Recovery.               |
|----------------------------------------|---------------------------------------|-------------------------|
| 26.3%                                  | { 47.3% Zn.<br>4.6% Pb.<br>1.0% Ins.  | { 65.8% Zn.<br>8.5% Pb. |
| 10.0%                                  | { 41.9% Zn.<br>10.0% Pb.<br>3.8% Ins. | { 22.3% Zn.<br>7.1% Pb. |
| 19.4%                                  | { 4.1% Zn.<br>60.0% Pb.<br>11.5% Ins. | { 4.2% Zn.<br>82.2% Pb. |

105

110

115

The proportion of the original in the tailings was 44.2, assaying 3.3% Zn, 0.7% Pb.

It will be clearly seen from these examples that in the case of the sized product the bulk of the zinc was floated first, while the bulk of the lead was floated later, whereby a preferential or selective separation was obtained.

It is important to note that the results may be seriously interfered with if the proportion of solute or of frothing agent be excessive or insufficient; and from the above directions it will be obvious that a few simple preliminary tests will determine the best conditions.

125

130

What I claim as my invention and desire to secure by Letters Patent is:—

1. A process of concentrating ores containing mixed metalliferous minerals which 5 consists in sizing such an ore so as to obtain a plurality of products one of which is a graded product composed of particles of substantially the same size, and thereafter subjecting such graded product to froth flotation treatment so as to preferentially float one of the metalliferous minerals.

2. A process of concentrating ores containing mixed metalliferous minerals which 15 consists in sizing such an ore so as to obtain a plurality of products one of which is a graded product composed of particles of substantially the same size, and thereafter subjecting such graded product to froth flotation treatment so as to obtain a flotation product relatively high in a certain metalliferous mineral on the one hand and a residue relatively high in another metalliferous mineral on the other hand, and submitting the residue to further froth flotation 20 treatment for the recovery of the metalliferous mineral contained therein.

3. A process of concentrating ores containing mixed metalliferous minerals which 30 consists in sizing such an ore in a finely crushed condition into a plurality of grades each composed of particles of substantially the same size, and thereafter subjecting each grade separately to froth flotation treatment so as to preferentially float one of the metalliferous minerals.

4. A process of concentrating ores containing mixed metalliferous minerals which 40 consists in sizing such an ore in a finely crushed condition into a plurality of grades each composed of particles of substantially the same size, and thereafter subjecting each grade separately to froth flotation treatment so as to obtain flotation products relatively high in a certain metalliferous 45 mineral on the one hand and residues relatively high in another metalliferous mineral on the other hand, and submitting the residues to further froth flotation treatment for the recovery of the metalliferous mineral contained therein.

5. A process of concentrating ores containing mixed metalliferous minerals which 55 consists in sizing such an ore so as to obtain a plurality of products one of which is a graded product composed of particles of substantially the same size, and thereafter subjecting such graded product to froth flotation treatment with subaeration so as to preferentially float one of the metalliferous 60 minerals.

6. A process of concentrating ores containing mixed metalliferous minerals which 65 consists in sizing such an ore so as to obtain a plurality of products one of which is a graded product composed of particles of

substantially the same size, and thereafter subjecting such graded product to froth flotation treatment with subaeration so as to obtain a flotation product relatively high in a certain metalliferous mineral on the one 70 hand and a residue relatively high in another metalliferous mineral on the other hand, and submitting the residue to further froth flotation treatment for the recovery of the metalliferous mineral contained 75 therein.

7. A process of concentrating ores containing mixed metalliferous minerals which 80 consists in sizing such an ore in a finely crushed condition into a plurality of grades each composed of particles of substantially the same size, and thereafter subjecting each grade separately to froth flotation treatment with subaeration so as to preferentially float one of the metalliferous minerals. 85

8. A process of concentrating ores containing mixed metalliferous minerals which 90 consists in sizing such an ore in a finely crushed condition into a plurality of grades each composed of particles of substantially the same size, and thereafter subjecting each grade separately to froth flotation treatment with subaeration so as to obtain flotation products relatively high in a certain metalliferous mineral on the one hand and residues 95 relatively high in another metalliferous mineral on the other hand, and submitting the residues to further froth flotation treatment for the recovery of the metalliferous mineral contained therein. 100

9. A process of concentrating zinc-lead ores which consists in sizing such an ore so as to obtain a plurality of products one of which is a graded product composed of particles of substantially the same size, and 105 thereafter subjecting such graded product to froth flotation treatment so as to obtain a flotation product relatively high in zinc on the one hand and a residue relatively high in lead on the other hand. 110

10. A process of concentrating zinc-lead ores which consists in sizing such an ore so as to obtain a plurality of products one of which is a graded product composed of particles of substantially the same size, and thereafter subjecting such graded product to froth flotation treatment so as to obtain a flotation product relatively high in zinc on the one hand and a residue relatively high in lead on the other hand, and submitting the residue to further froth flotation treatment for the recovery of the zinc contained therein.

11. A process of concentrating zinc-lead ores which consists in sizing such an ore in a finely crushed condition into a plurality of grades each composed of particles of substantially the same size, and thereafter subjecting each grade separately to froth flotation treatment so as to obtain a flotation

product relatively high in zinc on the one hand and a residue relatively high in lead on the other hand.

12. A process of concentrating zinc-lead ores which consists in sizing such an ore in a finely crushed condition into a plurality of grades each composed of particles of substantially the same size, and thereafter subjecting each grade separately to froth flotation treatment so as to obtain a flotation product relatively high in zinc on the one hand and a residue relatively high in lead on the other hand, and submitting the residue to further froth flotation treatment for the recovery of the lead contained therein.
13. A process of concentrating zinc-lead ores which consists in sizing such an ore so as to obtain a plurality of products one of which is a graded product composed of particles of substantially the same size, and thereafter subjecting such graded product to froth flotation treatment with subaeration so as to obtain a flotation product relatively high in zinc on the one hand and a residue relatively high in lead on the other hand.

14. A process of concentrating zinc-lead ores which consists in sizing such an ore so as to obtain a plurality of products one of which is a graded product composed of particles of substantially the same size, and thereafter subjecting such graded product to froth flotation treatment with subaeration so as to obtain a flotation product relatively high in zinc on the one hand and a residue relatively high in lead on the other hand, and submitting the residue to further froth flotation treatment for the recovery of the zinc contained therein.
15. A process of concentrating zinc-lead ores which consists in sizing such an ore in

a finely crushed condition into a plurality of grades each composed of particles of substantially the same size, and thereafter subjecting each grade separately to froth flotation treatment with subaeration so as to obtain a flotation product relatively high in zinc on the one hand and a residue relatively high in lead on the other hand. 45

16. A process of concentrating zinc-lead ores which consists in sizing such an ore in a finely crushed condition into a plurality of grades each composed of particles of substantially the same size, and thereafter subjecting each grade separately to froth flotation treatment with subaeration so as to obtain a flotation product relatively high in zinc on the one hand and a residue relatively high in lead on the other hand, and submitting the residue to further froth flotation treatment for the recovery of the lead contained therein. 50

17. A process of concentrating zinc-lead ores which consists in sizing such an ore so as to obtain a plurality of products one of which is a graded product composed of particles of substantially the same size, and thereafter subjecting such graded product to froth flotation treatment with subaeration in the presence of a minute quantity of 65 eucalyptus oil so as to obtain a flotation product relatively high in zinc on the one hand and a residue relatively high in lead on the other hand. 70

In testimony whereof I have signed my 75 name to this specification in the presence of two subscribing witnesses.

ARTHUR HOWARD HIGGINS.

Witnesses:

WILLIAM JAMES WALTON,  
GEORGE BUTTON.